

## UNITED STATES PATENT OFFICE

2,210,504

## LEAD ALLOY BEARING METAL

Robert J. Shoemaker, Chicago, Ill.

No Drawing. Application August 15, 1938,  
Serial No. 224,994

2 Claims. (Cl. 75—167)

This invention relates to hardened lead alloys having characteristics making them suitable for bearings.

The primary hardening agent is calcium and it is used in amounts sufficient so that a relatively large number of calcium-lead crystals  $Pb_3Ca$  are produced, which give the alloy its capacity for withstanding wear and resisting impact necessary to make the alloy useable for certain types 10 of bearings. That is, the calcium is used in such quantity that a minor portion of it (less than 0.1%) goes into solid solution with the lead, and a major portion forms the before-mentioned calcium-lead crystals.

15 The alloy radically differs from the bearing alloy described and claimed in United States patents to Robert J. Shoemaker, Nos. 1,745,721; 1,808,793 and 1,916,496, in which lithium, and potassium are variously employed as hardening agents, since it has been found that those ingredients imparted deleterious corrosive effect to the alloy, particularly when used in thin bearing linings where the alloy may be only 1/32 inch to 1/16 inch thick, as in bearings for automobiles, 20 Diesel engines, and the like. It has also been found that potassium and lithium are rather unstable and drop off readily on remelts.

25 The instant invention contemplates, not merely the use of as high as 2.0% calcium, but the avoidance of the use of lithium, and potassium, without the loss of the desirable characteristics usually imparted to alloys thereby.

The alloy differs radically in its characteristics from the lead alloy intended particularly for 30 cable coverings, pipes, and like articles described and claimed in patent to Robert J. Shoemaker, No. 1,813,324, patented July 7, 1931, in which such small quantities of calcium are used that either all of it goes into solid solution with the lead or the calcium-lead crystals formed are so small 35 in number and size, and consequently are so widely distributed in the body of the alloy, that they add substantially nothing to the wear or impact resistance qualities of the alloy.

40 The present invention also contemplates the use of secondary hardeners such as tin and mercury, the employment of which latter, however, is optional; and, as mercury is poisonous and to 45 some extent dangerous if used in large quantities

for the purpose of enhancing the hardness of the alloy, the present invention contemplates the use of other secondary hardeners in place of all or part of the mercury, to wit, silver, magnesium, barium, strontium, copper, manganese, in quantities to be indicated.

A preferred formula is as follows, percentages being by weight of the alloy, taking into account, so far as possible, oxidation and other compounding losses:

|          | Percent |
|----------|---------|
| Calcium  | 0.6     |
| Tin      | 1.0     |
| Mercury  | 0.25    |
| Aluminum | 0.05    |
| Lead     | Balance |

These preferred quantities may be varied as follows:

|          | Percent      |
|----------|--------------|
| Calcium  | 0.6 to 2.0   |
| Tin      | 0.5 to 1.0   |
| Mercury  | 0.1 to 1.0   |
| Aluminum | 0.02 to 0.15 |
| Lead     | Balance      |

If the calcium is used in quantities above 2.0%, the alloy when melted will be too viscous. If the tin is used in quantities above 1.0%, the alloy becomes too brittle, the hardness is decreased, 30 and the melting point is reduced. If the mercury is used in quantities above 1.0%, it will volatilize.

The aluminum is optional, but practically necessary if the alloy is to be remelted. It is an anti-drossing agent preventing oxidation of the calcium. Since it is largely customary in the industry to remelt bearings of this type, it is also necessary to keep the barium content not in excess of 0.1% as in excess of that amount will 35 render the alloy unstable.

The use of mercury in excess of 1.0% will add considerably to the hardness of the alloy. For example, the hardness of the alloy made in accordance with the preferred formula given above, is about 20° on the Brinell scale with the metal at 70° Fahrenheit. The hardness may be increased to 25° by using mercury up to 1.0%; but the employment of mercury in this quantity is likely to result in the production of poisonous 40 45 50

fumes in the compounding or remelting of the alloy. To avoid this, where a high degree of hardness is desired, it is possible to employ, in place of the mercury, (or in addition to mercury in quantities from 0.1% to 0.25%) any of the following metals in the quantities indicated:

|              | Per cent     |
|--------------|--------------|
| Silver       | 0.5 to 2.0   |
| Barium       | 0.02 to 0.1  |
| 10 Strontium | 0.02 to 0.5  |
| Copper       | 0.05 to 0.5  |
| Manganese    | 0.05 to 0.5  |
| Magnesium    | 0.01 to 0.15 |

15 The method of compounding the alloy is as follows: The lead is melted and heated to a temperature of approximately 1500° Fahrenheit under a covering of calcium chloride or other suitable flux. The aluminum is introduced, preferably as an alloy consisting of 50% aluminum and 20 50% tin by weight. Since the amount of aluminum is very small, the tin introduced in this way is practically negligible. The calcium is introduced as metallic calcium or as an alloy consisting preferably of approximately 5% calcium 25 and 95% lead by weight. If any of the auxiliary hardeners, silver, barium, strontium, magnesium, copper or manganese are employed, it may be introduced at this stage, either as the pure metal or in the form of a tin alloy. The melt is then 30 allowed to cool to a temperature just above the melting point of lead, say to 700° Fahrenheit and the calcium-chloride covering is skimmed off; or the bath can be allowed to solidify and then remelted to about 700° Fahrenheit, whereupon, 35 in either case the mercury and tin are added.

Another preferred formula in compounding this alloy is as follows:

|          | Per cent |
|----------|----------|
| Calcium  | 0.8      |
| 40 Tin   | 1.0      |
| Mercury  | 0.25     |
| Aluminum | 0.05     |
| Lead     | Balance  |

and any one of the following in the amounts specified:

|           | Per cent |
|-----------|----------|
| Silver    | 1.0      |
| Magnesium | 0.05     |
| Barium    | 0.05     |
| Strontium | 0.25     |
| Copper    | 0.25     |
| Manganese | 0.25     |

10 The alloy of the preferred formula will have a hardness of 24° Brinell, a tensile strength of 12,000 pounds per square inch and an elongation of 9 to 12% of two inches.

It is thought that the invention and many of its attendant advantages will be understood from the foregoing description, and it will be apparent that various changes may be made in the formulae herein disclosed and described without departing from the spirit and scope of the invention or sacrificing all of its material advantages, the formulae hereinbefore disclosed being merely a preferred embodiment thereof.

I claim:

1. A hardened lead alloy for bearings containing, in addition to a main body of lead, a primary hardener comprising 0.6 to 2.0% of calcium; secondary hardeners comprising 0.5 to 1.0% of tin, and less than 1.0% of mercury, and a further hardening agent selected from a group comprising 0.5 to 2.0% of silver and 0.05 to 0.5% of copper; and an anti-drossing agent comprising 0.02 to 0.15% of aluminum.

2. A hardened lead alloy for bearings containing, in addition to a main body of lead, the following substances in quantities by weight substantially as follows: 0.8% of calcium; secondary hardeners comprising 1.0% of tin, .25% of mercury, and another hardening agent selected from a group composed of 1.0% silver and 0.25% of copper; and an anti-drossing agent comprising 0.05% of aluminum.

ROBERT J. SHOEMAKER.